



US007323071B1

(12) **United States Patent**  
**Branagan**

(10) **Patent No.:** **US 7,323,071 B1**  
(45) **Date of Patent:** **\*Jan. 29, 2008**

(54) **METHOD FOR FORMING A HARDEDED SURFACE ON A SUBSTRATE**

(75) Inventor: **Daniel J. Branagan**, Iona, ID (US)

(73) Assignee: **Battelle Energy Alliance, LLC**, Idaho Falls, ID (US)

(\*) Notice: Subject to any disclaimer, the term of this patent is extended or adjusted under 35 U.S.C. 154(b) by 371 days.

This patent is subject to a terminal disclaimer.

(21) Appl. No.: **10/841,873**

(22) Filed: **May 6, 2004**

**Related U.S. Application Data**

(63) Continuation of application No. 09/709,918, filed on Nov. 9, 2000, now Pat. No. 6,767,419.

(51) **Int. Cl.**  
**C21D 9/00** (2006.01)

(52) **U.S. Cl.** ..... **148/561**; 427/456

(58) **Field of Classification Search** ..... 148/561  
See application file for complete search history.

(56) **References Cited**

**U.S. PATENT DOCUMENTS**

|               |         |                  |         |
|---------------|---------|------------------|---------|
| 4,133,679 A * | 1/1979  | Ray              | 148/403 |
| 4,210,443 A * | 7/1980  | Ray              | 148/403 |
| 4,606,977 A * | 8/1986  | Dickson et al.   | 428/553 |
| 4,725,512 A   | 2/1988  | Scruggs          |         |
| 4,820,141 A   | 4/1989  | Shingu et al.    |         |
| 4,881,989 A * | 11/1989 | Yoshizawa et al. | 148/302 |
| 5,032,469 A   | 7/1991  | Merz et al.      |         |
| 5,376,191 A   | 12/1994 | Roman et al.     |         |

|                |        |                        |
|----------------|--------|------------------------|
| 5,643,531 A    | 7/1997 | Kim et al.             |
| 6,258,185 B1   | 7/2001 | Branagan et al.        |
| 6,261,386 B1   | 7/2001 | Perepezko et al.       |
| 6,270,591 B2   | 8/2001 | Chiriac et al.         |
| 6,767,419 B1 * | 7/2004 | Branagan ..... 148/522 |

**OTHER PUBLICATIONS**

Heffelfinger, R.E. et al., "Analysis of High-Purity Iron", Analytical Chemistry, Battelle Memorial Institute, Columbus, Ohio, p. 112, published in 1958.\*

Kamenetskaya, D.S. et al., "Notch Toughness of High-Purity Iron", Translated from Metallovedenie i Termicheskaya Obrabotka Metallov, No. 3, pp. 15-16, Mar. 1976, pp. 205-206.\*

Osinkolu, G.A. et al., "Hot Tensile Deformation of Ultra High Purity Iron Base Alloys Containing Al,N,S on Cooling to Test Temperatures", Scripta Materialia, vol. 36, No. 10, 1997, pp. 1139-1143.\*

Ide, K. et al., "Determination of Trace Refractory Metal Elements in High-Purity Iron by Inductively Coupled Plasma Mass Spectrometry", Japan Analyst, vol. 52, No. 10, 2003, Abstract only (2pp).\*

\* cited by examiner

*Primary Examiner*—George Wyszomierski

(74) **Attorney, Agent, or Firm**—Wells St. John P.S.

(57) **ABSTRACT**

The invention encompasses a method of forming a metallic coating. A metallic glass coating is formed over a metallic substrate. After formation of the coating, at least a portion of the metallic glass can be converted into a crystalline material having a nanocrystalline grain size. The invention also encompasses metallic coatings comprising metallic glass. Additionally, the invention encompasses metallic coatings comprising crystalline metallic material, with at least some of the crystalline metallic material having a nanocrystalline grain size.

**12 Claims, 18 Drawing Sheets**





II II II II





π π π 3



π π π 2

100



π π π 5

100



π π π 6

100



EE EE EE EE



5  $\mu\text{m}$

EE EE EE





ILLUSTRATION



**A: Gas Atomized Powder Particles**



**B: Melt-Spun Ribbon**



EX-07 12



FIG 6 FIG 7











787-001











## 1

METHOD FOR FORMING A HARDENED  
SURFACE ON A SUBSTRATE

## RELATED APPLICATIONS

This application is a continuation of U.S. patent application Ser. No. 09/709,918 filed on Nov. 9, 2000 now U.S. Pat. No. 6,767,419.

## CONTRACTUAL ORIGIN OF THE INVENTION

This invention was made with United States Government support under Contract No. DE-AC07-99ID13727 awarded by the United States Department of Energy. The United States Government has certain rights in the invention.

## TECHNICAL FIELD

The invention pertains to metallic coatings and methods of forming metallic coatings.

## BACKGROUND OF THE INVENTION

Steel is a metallic alloy which can have exceptional strength characteristics, and which is accordingly commonly utilized in structures where strength is required or advantageous. Steel can be utilized, for example, in the skeletal supports of building structures, tools, engine components, and protective shielding of modern armaments.

The composition of steel varies depending on the application of the alloy. For purposes of interpreting this disclosure and the claims that follow, "steel" is defined as any iron-based alloy in which no other single element (besides iron) is present in excess of 30 weight percent, and for which the iron content amounts to at least 55 weight percent, and carbon is limited to a maximum of 2 weight percent. In addition to iron, steel alloys can incorporate, for example, manganese, nickel, chromium, molybdenum, and/or vanadium. Steel alloys can also incorporate carbon, silicon, phosphorus and/or sulfur. However, phosphorus, carbon, sulfur and silicon can be detrimental to overall steel quality if present in quantities greater than a few percent. Accordingly, steel typically contains small amounts of phosphorus, carbon, sulfur and silicon.

Steel comprises regular arrangements of atoms, with the periodic stacking arrangements forming 3-dimensional lattices which define the internal structure of the steel. The internal structure (sometimes called "microstructure") of conventional steel alloys is always metallic and polycrystalline (consisting of many crystalline grains).

Steel is typically formed by cooling a molten alloy. The rate of cooling will determine whether the alloy cools to form an internal structure that predominately comprises crystalline grains, or, in rare cases, a structure which is predominately amorphous (a so-called metallic glass). Generally, it is found that if the cooling proceeds slowly (i.e., at a rate less than about  $10^4$  K/s), large grain sizes occur, while if the cooling proceeds rapidly (i.e., at a rate greater than or equal to about  $10^4$  K/s) microcrystalline internal grain structures are formed, or, in specific rare cases amorphous metallic glasses are formed. The particular composition of the molten alloy generally determines whether the alloy solidifies to form microcrystalline grain structures or an amorphous glass when the alloy is cooled rapidly. Also, it is noted that particular alloy compositions (not iron based) have recently been discovered which can lead to micro-

## 2

scopic grain formation, or metallic glass formation, at relatively low cooling rates (cooling rates on the order of 10 K/s).

Both microcrystalline grain internal structures and metallic glass internal structures can have properties which are desirable in particular applications for steel. In some applications, the amorphous character of metallic glass can provide desired properties. For instance, some glasses can have exceptionally high strength and hardness. In other applications, the particular properties of microcrystalline grain structures are preferred. Frequently, if the properties of a grain structure are preferred, such properties will be improved by decreasing the grain size. For instance, desired properties of microcrystalline grains (i.e., grains having a size on the order of  $10^{-6}$  meters) can frequently be improved by reducing the grain size to that of nanocrystalline grains (i.e., grains having a size on the order of  $10^{-9}$  meters). It is generally more problematic to form grains of nanocrystalline grain size than it is to form grains of microcrystalline grain size. Accordingly, it is desirable to develop improved methods for forming nanocrystalline grain size steel materials. Further, as it is frequently desired to have metallic glass structures, it is desirable to develop methods of forming metallic glasses.

## SUMMARY OF THE INVENTION

In one aspect, the invention encompasses a method of forming a metallic coating. A metallic glass coating is formed over a metallic substrate. After formation of the coating, at least a portion of the metallic glass can be converted into a crystalline material having a nanocrystalline grain size.

In another aspect, the invention encompasses metallic coatings comprising metallic glass.

In yet another aspect, the invention encompasses metallic coatings comprising crystalline metallic material, with at least some of the crystalline metallic material having a nanocrystalline grain size.

## BRIEF DESCRIPTION OF THE DRAWINGS

Preferred embodiments of the invention are described below with reference to the following accompanying drawings.

FIG. 1 is a block-diagram flowchart view of a method encompassed by the present invention.

FIG. 2 is a diagrammatic perspective view of a barrel being treated according to a method of the present invention.

FIG. 3 is a fragmentary, diagrammatic, cross-sectional view of a metallic material substrate at a preliminary step of a treatment process encompassed by the present invention.

FIG. 4 is a view of the FIG. 3 fragment shown at a processing step subsequent to that of FIG. 3.

FIG. 5 is a view of the FIG. 3 fragment shown at a processing step subsequent to that of FIG. 4.

FIG. 6 is a view of the FIG. 3 fragment shown at a processing step subsequent to that of FIG. 5.

FIG. 7 is an optical micrograph of a metallic glass ribbon formed in accordance with methodology of the present invention, and formed from a composition comprising  $Fe_{63}Cr_8Mo_2B_{17}C_5Si_1Al_4$ .

FIG. 8 is a scanning electron microscope micrograph of a cross section of a gas atomized powder particle formed in accordance with the present invention, and formed from a composition comprising  $Fe_{63}Cr_8Mo_2B_{17}C_5Si_1Al_4$ .

FIG. 9 is a graph illustrating the results of a differential thermal analysis scan of a ribbon produced in accordance with the present invention. The ribbon was produced from a composition comprising  $Fe_{63}Cr_8Mo_2B_{17}C_5Si_1Al_4$ . An exothermic glass to crystallization transition occurs at 550° C., and an endothermic solid to liquid melting transition occurs at 1,150° C.

FIG. 10 is a TEM micrograph of a steel alloy produced in accordance with the methodology of the present invention, and comprising a composition  $Fe_{63}Cr_8Mo_2B_{17}C_5Si_1Al_4$ , which has been heat treated for 650° C. for one hour. A nanoscale nanocomposite microstructure is visible, with phase sizes from 1 to 75 nanometers.

FIG. 11 illustrates Vickers hardness for different metallic alloys. Specifically, the figure compares DAR1 ( $Fe_{63}Cr_8Mo_2B_{17}C_5Si_1Al_4$ ) with DAR20 ( $Fe_{64}Ti_3Cr_5Mo_2B_{16}C_5Si_1Al_2La_2$ ). The hardness is compared as a function of heat treatment temperature.

FIG. 12 shows examples of Vickers hardness tests using a diamond pyramid indenter. Specifically, a top portion of the figure shows the test relative to gas atomized powder particles, and a lower portion shows the test utilized for a melt-spun ribbon. The tested composition was  $Fe_{63}Cr_8Mo_2B_{17}C_5Si_1Al_4$ .

FIG. 13 is an optical micrograph of a steel composition which has been plasma sprayed onto a stainless steel substrate. The plasma-sprayed steel composition comprises  $Fe_{63}Cr_8Mo_2B_{17}C_5Si_1Al_4$ . The top portion of FIG. 9(a) is a cross-sectional view of the sprayed material, and the lower portion (b) shows a top surface of the coated material.

FIG. 14 illustrates an x-ray diffraction scan of a plasma-sprayed deposit having a free surface. The plasma-sprayed composition was  $Fe_{63}Cr_8Mo_2B_{17}C_5Si_1Al_4$ .

FIG. 15 shows an x-ray diffraction scan of the plasma-sprayed composition of FIG. 14, and illustrates the structure at the substrate surface.

FIG. 16 illustrates a graph showing coefficient of friction versus the number of turns for Pin On Disk testing of a spray coating. The tested coating was  $Fe_{63}Cr_8Mo_2B_{17}C_5Si_1Al_4$ . It is noted that while the initial friction was low,  $Si_3N_4$  deposition and buildup caused the friction to increase. (The sliding friction of  $Si_3N_4$  on itself is 0.8).

FIG. 17 is a profile curve of a “wear-groove” on an as-sprayed steel substrate after 2,000 cycles of Pin On Disk testing. As shown, instead of a groove developing on the steel substrate, the  $Si_3N_4$  wore and deposited material onto the substrate. The tested composition was  $Fe_{63}Cr_8Mo_2B_{17}C_5Si_1Al_4$ .

FIG. 18 is an optical micrograph of an as-spun ribbon of ( $Fe_{0.8}Cr_{0.2}$ )<sub>81</sub> $B_{17}W_2$ . The alloy exhibits high ductility, and can be bent severely without fracture.

FIG. 19 illustrates data obtained from differential thermal analysis of ( $Fe_{0.8}Cr_{0.2}$ )<sub>75</sub> $B_{17}Si_4Al_4$  (top graph) and  $Fe_{63}Cr_8Mo_2B_{17}C_5Si_1Al_4$  (lower graph). The graph curves show glass to crystalline transitions and melting temperatures for the tested alloys.

FIG. 20 shows peak crystallization temperatures measured by differential thermal analysis for a variety of alloys. Specifically, FIG. 20 shows the alloy  $Fe_{63}Cr_8Mo_2B_{17}C_5Si_1Al_4$  as 1, ( $Fe_{0.85}Cr_{0.15}$ )<sub>83</sub> $B_{17}$  as 2, ( $Fe_{0.8}Cr_{0.2}$ )<sub>83</sub> $B_{17}$  as 3, ( $Fe_{0.75}Cr_{0.25}$ )<sub>83</sub> $B_{17}$  as 4, ( $Fe_{0.8}Mo_{0.2}$ )<sub>83</sub> $B_{17}$  as 5, ( $Fe_{0.6}Co_{0.2}Cr_{0.2}$ )<sub>83</sub> $B_{17}$  as 6, ( $Fe_{0.8}Cr_{0.15}Mo_{0.05}$ )<sub>83</sub> $B_{17}$  as 7, ( $Fe_{0.8}Cr_{0.2}$ )<sub>79</sub> $B_{17}C_4$  as 8, ( $Fe_{0.8}Cr_{0.2}$ )<sub>79</sub> $B_{17}Si_4$  as 9, ( $Fe_{0.8}Cr_{0.2}$ )<sub>79</sub> $B_{17}Al_4$  as 10, ( $Fe_{0.8}Cr_{0.2}$ )<sub>75</sub> $B_{17}Al_4C_4$  as 11, ( $Fe_{0.8}Cr_{0.2}$ )<sub>75</sub> $B_{17}Si_4C_4$  as 12, ( $Fe_{0.8}Cr_{0.2}$ )<sub>75</sub> $B_{17}Si_4Al_4$  as 13, ( $Fe_{0.8}Cr_{0.2}$ )<sub>71</sub> $B_{17}Si_4C_4Al_4$  as 14, ( $Fe_{0.7}Co_{0.1}Cr_{0.2}$ )<sub>83</sub> $B_{17}$  as 15, ( $Fe_{0.8}Cr_{0.2}$ )<sub>76</sub> $B_{17}Al_7$  as 16, ( $Fe_{0.8}Cr_{0.2}$ )<sub>79</sub> $B_{17}W_2C_2$  as 17, ( $Fe_{0.8}Cr_{0.2}$ )<sub>81</sub> $B_{17}W_2$  as 18 and ( $Fe_{0.8}Cr_{0.2}$ )<sub>80</sub> $B_{20}$  as 19.

14, ( $Fe_{0.7}Co_{0.8}Cr_{0.2}$ )<sub>83</sub> $B_{17}$  as 15, ( $Fe_{0.8}Cr_{0.2}$ )<sub>76</sub> $B_{17}Al_7$  as 16, ( $Fe_{0.8}Cr_{0.2}$ )<sub>79</sub> $B_{17}W_2C_2$  as 17, ( $Fe_{0.8}Cr_{0.2}$ )<sub>81</sub> $B_{17}W_2$  as 18 and ( $Fe_{0.8}Cr_{0.2}$ )<sub>80</sub> $B_{20}$  as 19.

FIG. 21 illustrates crystallization enthalpies measured by differential scanning calorimetry for various alloys encompassed by the present invention. Specifically, FIG. 21 shows the alloy  $Fe_{63}Cr_8Mo_2B_{17}C_5Si_1Al_4$  as 1, ( $Fe_{0.85}Cr_0O_{15}$ )<sub>83</sub> $B_{17}$  as 2, ( $Fe_{0.8}Cr_{0.2}$ )<sub>83</sub> $B_{17}$  as 3, ( $Fe_{0.75}Cr_{0.25}$ )<sub>83</sub> $B_{17}$  as 4, ( $Fe_{0.8}Mo_{0.2}$ )<sub>83</sub> $B_{17}$  as 5, ( $Fe_{0.6}Co_{0.2}Cr_{0.2}$ )<sub>83</sub> $B_{17}$  as 6, ( $Fe_{0.8}Cr_{0.15}Mo_{0.05}$ )<sub>83</sub> $B_{17}$  as 7, ( $Fe_{0.8}Cr_{0.2}$ )<sub>79</sub> $B_{17}C_4$  as 8, ( $Fe_{0.8}Cr_{0.2}$ )<sub>79</sub> $B_{17}Si_4$  as 9, ( $Fe_{0.8}Cr_{0.2}$ )<sub>79</sub> $B_{17}Al_4$  as 10, ( $Fe_{0.8}Cr_{0.2}$ )<sub>75</sub> $B_{17}Al_4C_4$  as 11, ( $Fe_{0.8}Cr_{0.2}$ )<sub>75</sub> $B_{17}Si_4C_4$  as 12, ( $Fe_{0.8}Cr_{0.2}$ )<sub>75</sub> $B_{17}Si_4Al_4$  as 13, ( $Fe_{0.8}Cr_{0.2}$ )<sub>71</sub> $B_{17}Si_4C_4Al_4$  as 14, ( $Fe_{0.7}Co_{0.1}Cr_{0.2}$ )<sub>83</sub> $B_{17}$  as 15, ( $Fe_{0.8}Cr_{0.2}$ )<sub>76</sub> $B_{17}Al_7$  as 16, ( $Fe_{0.8}Cr_{0.2}$ )<sub>79</sub> $B_{17}W_2C_2$  as 17, ( $Fe_{0.8}Cr_{0.2}$ )<sub>81</sub> $B_{17}W_2$  as 18 and ( $Fe_{0.8}Cr_{0.2}$ )<sub>80</sub> $B_{20}$  as 19.

FIG. 22 illustrates a graph of transformation rates of glass to crystallization transformation for various alloys encompassed by the present invention. Specifically, FIG. 22 shows the alloy  $Fe_{63}Cr_8Mo_2B_{17}C_5Si_1Al_4$  as 1, ( $Fe_{0.85}Cr_{0.15}$ )<sub>83</sub> $B_{17}$  as 2, ( $Fe_{0.8}Cr_{0.2}$ )<sub>83</sub> $B_{17}$  as 3, ( $Fe_{0.75}Cr_{0.25}$ )<sub>83</sub> $B_{17}$  as 4, ( $Fe_{0.8}Mo_{0.2}$ )<sub>83</sub> $B_{17}$  as 5, ( $Fe_{0.6}Co_{0.2}Cr_{0.2}$ )<sub>83</sub> $B_{17}$  as 6, ( $Fe_{0.8}Cr_{0.15}Mo_{0.05}$ )<sub>83</sub> $B_{17}$  as 7, ( $Fe_{0.8}Cr_{0.2}$ )<sub>79</sub> $B_{17}C_4$  as 8, ( $Fe_{0.8}Cr_{0.2}$ )<sub>79</sub> $B_{17}Si_4$  as 9, ( $Fe_{0.8}Cr_{0.2}$ )<sub>79</sub> $B_{17}Al_4$  as 10, ( $Fe_{0.8}Cr_{0.2}$ )<sub>75</sub> $B_{17}Al_4C_4$  as 11, ( $Fe_{0.8}Cr_{0.2}$ )<sub>75</sub> $B_{17}Si_4C_4$  as 12, ( $Fe_{0.8}Cr_{0.2}$ )<sub>75</sub> $B_{17}Si_4Al_4$  as 13, ( $Fe_{0.8}Cr_{0.2}$ )<sub>71</sub> $B_{17}Si_4C_4Al_4$  as 14, ( $Fe_{0.7}Co_{0.1}Cr_{0.2}$ )<sub>83</sub> $B_{17}$  as 15, ( $Fe_{0.8}Cr_{0.2}$ )<sub>76</sub> $B_{17}Al_7$  as 16, ( $Fe_{0.8}Cr_{0.2}$ )<sub>79</sub> $B_{17}W_2C_2$  as 17, ( $Fe_{0.8}Cr_{0.2}$ )<sub>81</sub> $B_{17}W_2$  as 18 and ( $Fe_{0.8}Cr_{0.2}$ )<sub>80</sub> $B_{20}$  as 19.

FIG. 23 illustrates peak melting temperatures measured by differential thermal analysis for various alloys encompassed by the present invention. Specifically, FIG. 23 shows the alloy  $Fe_{63}Cr_8Mo_2B_{17}C_5Si_1Al_4$  as 1, ( $Fe_{0.85}Cr_{0.15}$ )<sub>83</sub> $B_{17}$  as 2, ( $Fe_{0.8}Cr_{0.2}$ )<sub>83</sub> $B_{17}$  as 3, ( $Fe_{0.75}Cr_{0.25}$ )<sub>83</sub> $B_{17}$  as 4, ( $Fe_{0.8}Mo_{0.2}$ )<sub>83</sub> $B_{17}$  as 5, ( $Fe_{0.6}Co_{0.2}Cr_{0.2}$ )<sub>83</sub> $B_{17}$  as 6, ( $Fe_{0.8}Cr_{0.15}Mo_{0.05}$ )<sub>83</sub> $B_{17}$  as 7, ( $Fe_{0.8}Cr_{0.2}$ )<sub>79</sub> $B_{17}C_4$  as 8, ( $Fe_{0.8}Cr_{0.2}$ )<sub>79</sub> $B_{17}Si_4$  as 9, ( $Fe_{0.8}Cr_{0.2}$ )<sub>79</sub> $B_{17}Al_4$  as 10, ( $Fe_{0.8}Cr_{0.2}$ )<sub>75</sub> $B_{17}Al_4C_4$  as 11, ( $Fe_{0.8}Cr_{0.2}$ )<sub>75</sub> $B_{17}Si_4C_4$  as 12, ( $Fe_{0.8}Cr_{0.2}$ )<sub>75</sub> $B_{17}Si_4Al_4$  as 13, ( $Fe_{0.8}Cr_{0.2}$ )<sub>71</sub> $B_{17}Si_4C_4Al_4$  as 14, ( $Fe_{0.7}Co_{0.1}Cr_{0.2}$ )<sub>83</sub> $B_{17}$  as 15, ( $Fe_{0.8}Cr_{0.2}$ )<sub>76</sub> $B_{17}Al_7$  as 16, ( $Fe_{0.8}Cr_{0.2}$ )<sub>79</sub> $B_{17}W_2C_2$  as 17, ( $Fe_{0.8}Cr_{0.2}$ )<sub>81</sub> $B_{17}W_2$  as 18 and ( $Fe_{0.8}Cr_{0.2}$ )<sub>80</sub> $B_{20}$  as 19.

## DETAILED DESCRIPTION OF THE PREFERRED EMBODIMENTS

This disclosure of the invention is submitted in furtherance of the constitutional purposes of the U.S. Patent Laws “to promote the progress of science and useful arts” (Article 1, Section 8).

The invention encompasses methodology for forming steel materials having nanocrystalline scale composite microstructures, methods of utilizing such steel materials, and also encompasses the steel material compositions. A process encompassed by the present invention is described generally with reference to the block diagram of FIG. 1. At an initial step (A) a molten alloy is formed. Such alloy comprises a steel composition. An exemplary alloy comprises at least 50% Fe and at least one element selected from the group consisting of Ti, Zr, Hf, V, Nb, Ta, Cr, Mo, W, Al, La, Ce, Pr, Nd, Sm, Eu, Gd, Tb, Dy, Ho, Er, Tm, Yb, and Lu; and at least one element selected from the group consisting of B, C, N, O, P and S. In particular aspects of the present invention, the alloy will be a magnetic alloy with ultrafine crystal grains having a composition represented by the formula:  $Fe(100-x-y)M(x)B(y)$  (atomic percent) wherein M represents at least one element selected from Ti, Zr, Hf,

5

V, Nb, Mo, Ta, Cr, W and Mn, wherein  $15 \leq x \leq 4$ , wherein  $25 \leq y \leq 2$ , and wherein  $35 \leq (x+y) \leq 7$ . Also, at least 50% of the alloy structure is preferably occupied by crystal grains having an average size of 1000 Å or less, with the crystal grains being based on a bcc structure. The alloy can further contain X (Si, Ge, P, Ga, etc.) and/or T (Au, Co, Ni, etc.).

Alloys of the present invention preferably comprise fewer than 11 elements, and can more preferably comprise fewer than seven elements. Additionally, the alloys can comprise fewer than five elements. An advantage in having fewer elements in the compositions is that it can be easier to reproduce a material if fewer components are utilized in forming the material. Generally, alloys of the present invention have from four to six elements in their compositions. Among such elements are iron; chromium, which can be included for corrosion resistance; boron and/or phosphorus which can be included to generate a particular glass transition temperature; and one or both of molybdenum and tungsten which can be included for hardness.

Exemplary alloys which can be utilized in methodology of the present invention are:  $(Fe_{0.85}Cr_{0.15})_{83}B_{17}$ ,  $(Fe_{0.8}Cr_{0.2})_{83}B_{17}$ ,  $(Fe_{0.75}Cr_{0.25})_{83}B_{17}$ ,  $(Fe_{0.8}Mo_{0.2})_{83}B_{17}$ ,  $(Fe_{0.6}Co_{0.2}Cr_{0.2})_{83}B_{17}$ ,  $(Fe_{0.8}Cr_{0.15}Mo_{0.05})_{83}B_{17}$ ,  $(Fe_{0.8}Cr_{0.2})_{79}B_{17}C_4$ ,  $(Fe_{0.8}Cr_{0.2})_{79}B_{17}Si_4$ ,  $(Fe_{0.8}Cr_{0.2})_{79}B_{17}Al_4$ ,  $(Fe_{0.8}Cr_{0.2})_{75}B_{17}Al_4C_4$ ,  $(Fe_{0.8}Cr_{0.2})_{75}B_{17}Si_4C_4$ ,  $(Fe_{0.8}Cr_{0.2})_{75}B_{77}Si_4Al_4$ ,  $(Fe_{0.8}Cr_{0.2})_{71}B_{17}Si_4C_4Al_4$ ,  $(Fe_{0.7}Co_{0.1}Cr_{0.2})_{83}B_7$ ,  $(Fe_{0.8}Cr_{0.2})_{76}B_{17}Al_7$ ,  $(Fe_{0.8}Cr_{0.2})_{79}B_{17}W_2C_2$ ,  $(Fe_{0.8}Cr_{0.2})_{81}B_{17}W_2$ , and  $(Fe_{0.8}Cr_{0.2})_{80}B_{20}$ .

The alloy of step (A) can be formed by, for example, melting a composition under an argon atmosphere.

At step (B) of FIG. 1, the alloy is cooled to form a metallic glass. Such cooling typically comprises a rate of at least about  $10^4$  K/s, with the rate varying depending on the particular composition of the molten alloy. The cooling can be accomplished by a number of different processes, including, for example, melt-spinning, gas atomization, centrifugal atomization, water atomization and splat quenching. The powder can be consolidated by, for example, hot pressing, hot extrusion, powder rolling, powder forging and dynamic compaction. In an exemplary method, the cooling of step (B) is accomplished by centrifugal atomization. Preferably, the melt stream leaves a centrifugal cup and is hit by high pressure helium gas to facilitate fast cooling (greater than  $10^5$  K/s.) The helium gas can be collected, purified and reused. The speed of the rotating centrifugal cup is preferably about 40,000 RPM, and such speed can be adjusted to produce a fine powder with about a 25 micrometer mean size.

Referring to step (C) of FIG. 1, the metallic glass of step (B) is devitrified to form a crystalline steel material having a nanocrystalline grain size. Such devitrification can be accomplished by heating the metallic glass to a temperature of from about 600° C. to less than the melting temperature of the alloy. Such heating enables a solid state phase change wherein the amorphous phase of the metallic glass is converted to one or more crystalline solid phases. The solid state devitrification of the amorphous precursor from step (B) enables uniform nucleation to occur throughout the metallic glass to form nanocrystalline grains within the glass. The metal matrix microstructure formed via the devitrification can comprise a steel matrix (iron with dissolved interstitials), with an intimate mixture of ceramic precipitates (transition metal carbides, borides, silicides, etc.). The nanocrystalline scale metal matrix composite grain structure can enable a combination of mechanical properties which are improved compared to the properties which would exist

6

with larger grain sizes or with the metallic glass. Such improved mechanical properties can include, for example, high strength, and high hardness coupled with significant ductility.

5 The particular temperature employed for devitrifying the metal glass can be varied depending on the particular alloy utilized in the glass, and a particular time of application.

Post treatment of the devitrified metallic material from step (C) can include a surface treatment utilized to transform only the surface of the material to a metallic glass. Exemplary surface treatment techniques are high and low pressure plasma spraying, high velocity oxyfuel spraying, and spray forming. The plasma spraying can be accomplished with a plasma spray system. The post treatment can offer improvements in, for example, corrosion resistance and lowering the coefficient of friction of a steel material. Accordingly, it can be advantageous to treat at least the surface of a crystalline steel material to convert such surface to a metallic glass. It is noted that a metallic glass coating can also offer advantages over existing coatings such as, for example, chrome, nickel and tin plating in that the metallic glass coating can be cheaper and can give a better metallurgical bond between the surface and the base metal.

Referring to FIG. 2, a specific embodiment application of the present invention is illustrated. Specifically, FIG. 2 illustrates a metallic barrel 50 being sprayed with a molten metal material 52. Molten metal material 52 is sprayed from a spraying device 54, and can comprise, for example, one or more of the above-described exemplary alloys of the present invention. The molten metal can be formed by melting an alloy composition under an argon atmosphere and subsequently centrifugally atomizing the alloy composition. As the melt stream leaves a centrifugal cup, it can be hit by a high pressure helium gas to form a fine powder of solidified metallic alloy material with such fine powder having about a 25 micrometer mean size. The fine powder can be fed into a plasma (high or low pressure) system wherein it is converted to a liquid spray which is sprayed on the inside and outside of metallic drum 50. In particular applications, drum 50 comprises a steel drum, such as, for example, a 55 gallon steel drum. It is noted that the powder may or may not be fully melted upon exposure to the plasma, and will be deposited into and onto the surface of barrel 50 as a continuous coating. In either event, the metallic material 52 sprayed onto and within drum 50 cools rapidly to form a metallic glass. Drum 50 can be subsequently heat-treated at a temperature of equal to or greater than 600° C. to devitrify the metallic glass.

The metallic structure formed over and within barrel 50 from material 52 can have greater corrosion resistance than stainless steel. Drum 50 be utilized, for example, for storing corrosive and otherwise dangerous materials, such as, for example, spent nuclear fuel. If a surface of material 52 is coated with a metallic glass, the anti-corrosive properties and low coefficient of friction properties associated with metallic glass can be obtained.

FIGS. 3-6 illustrate another embodiment application of the present invention. Referring to FIG. 3, a metallic substrate 100 is provided. Such substrate can comprise, for example, one or more of the above-described exemplary alloys of the present invention.

Referring to FIG. 4, a metallic melt **102** is sprayed onto substrate **100** utilizing a sprayer **104**. Melt **102** can comprise, for example, a molten alloy comprising one or more of  $(Fe_{0.85}Cr_{0.15})_{83}B_{17}$ ,  $(Fe_{0.8}Cr_{0.2})_{83}B_{17}$ ,  $(Fe_{0.75}Cr_{0.25})_{83}B_{17}$ ,  $(Fe_{0.8}Mo_{0.2})_{83}B_{17}$ ,  $(Fe_{0.6}Co_{0.2}Cr_{0.2})_{83}B_{17}$ ,  $(Fe_{0.8}Cr_{0.15}Mo_{0.05})_{83}B_{17}$ ,  $(Fe_{0.8}Cr_{0.2})_{79}B_{17}C_4$ ,  $(Fe_{0.8}$

$\text{Cr}_{0.2})_{79}\text{B}_{17}\text{Si}_4$ ,  $(\text{Fe}_{0.8}\text{Cr}_{0.2})_{79}\text{B}_{17}\text{Al}_4$ ,  $(\text{Fe}_{0.8}\text{Cr}_{0.2})_{75}\text{B}_{17}\text{Al}_4\text{C}_4$ ,  $(\text{Fe}_{0.8}\text{Cr}_{0.2})_{75}\text{B}_{17}\text{Si}_4\text{C}_4$ ,  $(\text{Fe}_{0.8}\text{Cr}_{0.2})_{75}\text{B}_{17}\text{Si}_4\text{Al}_4$ ,  $(\text{Fe}_{0.8}\text{Cr}_{0.2})_{71}\text{B}_{17}\text{Si}_4\text{C}_4\text{Al}_4$ ,  $(\text{Fe}_{0.7}\text{Co}_{0.1}\text{Cr}_{0.2})_{83}\text{B}_7$ ,  $(\text{Fe}_{0.8}\text{Cr}_{0.2})_{76}\text{B}_{17}\text{Al}_7$ ,  $(\text{Fe}_{0.8}\text{Cr}_{0.2})_{79}\text{B}_{17}\text{W}_2\text{C}_2$ ,  $(\text{Fe}_{0.8}\text{Cr}_{0.2})_{81}\text{B}_{17}\text{W}_2$ , and  $(\text{Fe}_{0.8}\text{Cr}_{0.2})_{80}\text{B}_{20}$ . Instead of being in a molten form, material 102 can alternatively comprise a powder material heated to a sufficient temperature to bond with the metal of layer 100.

Material 102 deposits on substrate 100 to form a layer 106. Material 102 also heats an exposed surface of material 100 to form a heat-treated portion 108 of material 100. If material 100 comprises a metallic glass, heat-treated portion 108 can comprise a devitrified material. Specifically, if layer 106 is formed at a temperature which heats a surface of layer 100 to greater than 600° C., such heating can devitrify a portion of material 100 exposed to such temperatures. In particular applications, temperatures greater than 600° C. can permeate entirely through substrate 100 to heat-treat an entire thickness of material 100. Spray nozzle 104 is preferably resistant to the temperature and composition of material 102.

Referring to FIG. 5, substrate 100 is illustrated after layer 106 has been formed across an entire surface of substrate 100. Heat-treated portion 108 also extends across an entire surface of substrate 100. In particular embodiments, layer 106 can be formed as a metallic glass.

Referring to FIG. 6, subsequent treatments of the type illustrated in FIG. 4 can be utilized to form multiple heat-treated layers 120 and an exposed outer surface layer 124. Note that one of the lower heat-treated layers 120 is previous layer 106. The subsequent formation of another metallic glass layer over layer 106 has heat-treated the entire layer 106. In particular embodiments wherein layer 106 comprises a metallic glass, such heat treatment can devitrify layer 106. Accordingly, heat treated layers 120 can comprise devitrified metal layers. In alternative methods of the present invention, each of the layers 106 and 120 can be deposited as metallic glass and can remain in the metallic glass form during deposition of remaining layers 120. Then, if desired, some or all of the deposited layers can be heat-treated to at least partially devitrify the coating defined by layers 106 and 120.

Outermost layer 124 may or may not be heat-treated, and can comprise a metallic glass. Accordingly, the method of the present invention has enabled an exterior coating to be formed over layer 100, with said exterior coating comprising devitrified metal layers 120 and an outermost surface of metallic glass 124.

The methodology described with reference to FIGS. 3-6 can have application for a number of uses, including military uses. Specifically, armor can be formed out of a material 100. If the armor becomes punctured or cracked, the methodology of FIGS. 3-6 can be utilized to repair the armor and effectively build a metallic shell over the weakened areas of the armor. Spraying device 104 can be adapted to be utilized in battlefield situations.

In addition to the utilizations described above for materials of the present invention, the materials can also be utilized as powders for surface finishing (i.e., mechanical blasting) and surface treatments such as, for example, shot peening.

The invention can be considered a method for forming a new class of steel called devitrified nanocomposite (DNC) steel, with DNC steel being defined as having a primarily nanoscale (less than 100 nanometer) microstructure grain size developed by processing the steel through a solid-solid transformation (specifically, glass devitrification). Alloys are

developed having low cooling rates (less than 10<sup>6</sup> K/s) for metallic glass formation, and accordingly the alloy compositions form metallic glasses when rapidly solidified by a chill surface (such as, for example, melt-spinning, splat quenching, etc.) or atomization (gas, water, centrifugal, etc.) methods. The glass is utilized as a precursor stage, and the alloy subsequently processed through a glass devitrification transformation upon heating above a crystallization temperature of the alloy. Due to uniform nucleation in the glass coupled with a high nucleation frequency, there is little time for grain growth processes, and nanoscale nanocomposite microstructures (i.e., grains) result. The nanocomposite microstructures can lead to materials having significant increases in hardness and strength over conventional steel alloys.

Initial studies described herein show that DNC steel formed in accordance with methodology of the present invention has exceptional hardness and wear resistance, and can be used potentially for any application which involves sliding, rolling, or rotation. Additionally, initial studies have shown that the unlubricated DNC steel surface has exceptionally low coefficients of friction (in the range of lubricated steels) which can be a beneficial property in reducing wear resistance, frictional energy losses, and heating between moving surfaces. This can allow the use of DNC steel in unlubricated applications, and can also be useful as a fail-safe mechanism allowing additional time before failure in some applications, such as gasoline or diesel engines, where lubrication is unexpectedly lost. The high wear resistance of DNC steel, coupled with low friction, can allow extension of the lifetime of parts formed from DNC steel relative to parts formed from conventional steel alloys. Such can enable large savings in both operating energy and cost associated with part replacement, repair, maintenance and down-time. Exemplary applications for utilization of DNC steels of the present invention include bearings, gun barrel surfaces, bearing journals, hydraulic cylinder connecting rods, crankshafts, pistons, cylinder liners, gears, camshafts, universal joints, valves, gun breach boxes, missile launcher tubes, and tank gear boxes.

Unlike conventional steel alloys which rely on manipulation of solid state eutectoid transformation ( $\gamma_{so} \rightleftharpoons \alpha_{so} + \text{Fe}_3\text{C}$ ), DNC steel utilizes a different approach, and specifically utilizes processing through a solid/solid state glass devitrification transformation. DNC steel alloys have been developed which have exceptionally low cooling rates (10<sup>3</sup> K/s to 10<sup>5</sup> K/s) for metallic glass formation. This can allow the production of metallic glass structures during rapid solidification via chill surface or atomization methods.

Examples of DNC steel melt-spun ribbon and gas atomized powder are shown in FIGS. 7 and 8, respectively. Metallic glass structures are produced by both of these rapid solidification processing methods. The glass precursor can be devitrified into a nanoscale composite microstructure by heating above the crystallization temperature.

A differential thermal analysis scan for as-spun DNC steel is shown in FIG. 9. The glass crystallization temperature typically varies from 750K to 900K with enthalpies of transformation from -75 J/g to -200 J/g, and melting temperatures from 1,375K to 1,500K for alloys encompassed by the present invention (as described in the charts of FIGS. 20-23). Because there is uniform nucleation and extremely high nucleation frequency during crystallization of alloys of the present invention, there can be little time for grain growth before impingement between neighboring

9 grains and accordingly nanoscale nanocomposite microstructures are formed. The individual phase sizes can vary from 1 to 75 nanometers, which is finer than conventional steels produced by conventional casting or even when rapidly solidified. When the microstructure is reduced to the nanoscale level, a high percentage of the atoms of the material (about 30%) can be associated with grain boundaries, and an extremely high density of two-dimensional defect interfaces (such as phase in grain boundaries) reside in the microstructure. The microstructure of a devitrified ribbon showing the nanoscale nanocomposite microstructure is shown in FIG. 10. The nanostructure results in the development of extreme strength and hardness, which are significantly higher than found in conventional steel or other metallic based alloys.

15 The hardness of glass and devitrified DNC steel has been measured using both nanoindentor and Vickers microhardness testing, and excellent agreement is found between the two methods. Specialized nanoindentor testing using a Berkovitch indenter was performed on the as-atomized and heat-treated sieved (10-20 micrometer and 75-100 micrometer) gas atomized particles from a  $Fe_{63}Cr_8Mo_2B_{17}C_5Si_1Al_4$  alloy as a function of depth into the particle. The elastic modulus was found to be as high as 300 GPa, which is approximately 50% higher than a conventional steel (which commonly exhibits elastic moduli from 200 GPa to 220 GPa). This means that bonding strength is increased, which can be of 20 beneficial result since it allows close tolerances to be maintained during application of high elastic loads, and can have additional benefits concerning wear resistance. The hardness was also found to be extremely high at greater than 15 GPa, which is harder than conventional metallic materials. Examples of various compositions which can be utilized in 25 methodology of the present invention for forming hard materials are shown in Table 1. In referring to Table, the various compositions are given reference names (specifically, they are referred to as alloys DARX) to simplify reference to the compositions herein. Table 2 contrasts 30 hardness of various materials with the alloy DAR1.

TABLE 1

DNC Alloy Compositions

| Alloy | Composition                                |
|-------|--------------------------------------------|
| DAR1  | $Fe_{63}Cr_8Mo_2B_{17}C_5Si_1Al_4$         |
| DAR2  | $(Fe_{0.82}Cr_{0.15})_{83}B_{17}$          |
| DAR3  | $(Fe_{0.8}Cr_{0.2})_{83}B_{17}$            |
| DAR4  | $(Fe_{0.75}Cr_{0.25})_{83}B_{17}$          |
| DAR5  | $(Fe_{0.8}Mo_{0.2})_{83}B_{17}$            |
| DAR6  | $(Fe_{0.6}Co_{0.2}Cr_{0.2})_{83}B_{17}$    |
| DAR7  | $(Fe_{0.8}Cr_{0.15}Mo_{0.05})_{83}B_{17}$  |
| DAR8  | $(Fe_{0.8}Cr_{0.2})_{79}B_{17}C_4$         |
| DAR9  | $(Fe_{0.8}Cr_{0.2})_{79}B_{17}Si_4$        |
| DAR10 | $(Fe_{0.8}Cr_{0.2})_{79}B_{17}Al_4$        |
| DAR11 | $(Fe_{0.8}Cr_{0.2})_{75}B_{17}Al_4C_4$     |
| DAR12 | $(Fe_{0.8}Cr_{0.2})_{75}B_{17}Si_4C_4$     |
| DAR13 | $(Fe_{0.8}Cr_{0.2})_{75}B_{17}Si_4Al_4$    |
| DAR14 | $(Fe_{0.8}Cr_{0.2})_{71}B_{17}Si_4C_4Al_4$ |
| DAR15 | $(Fe_{0.7}Co_{0.1}Cr_{0.2})_{83}B_{17}$    |
| DAR16 | $(Fe_{0.8}Cr_{0.2})_{76}B_{17}Al_7$        |
| DAR17 | $(Fe_{0.8}Cr_{0.2})_{79}B_{17}W_2C_2$      |
| DAR18 | $(Fe_{0.8}Cr_{0.2})_{81}B_{17}W_2$         |
| DAR19 | $(Fe_{0.8}Cr_{0.2})_{80}B_{20}$            |
| DAR20 | $Fe_{64}Ti_3Cr_5Mo_2B_{16}C_5Si_1Al_2La_2$ |

TABLE 2

| <u>Example Hardness of Metallic Materials</u> |                                           |          |
|-----------------------------------------------|-------------------------------------------|----------|
|                                               | Material                                  | Hardness |
| 5                                             | 18 Cr—10 Ni austenitic stainless steel    | 1.5 GPa  |
|                                               | 0.74 plain carbon steel                   | 4.9 GPa  |
|                                               | 4340 ultra high strength steel            | 5.5 GPa  |
|                                               | T5 W tool steel                           | 7.5 GPa  |
| 10                                            | 90 WC—10 Co cemented carbide              | 10.1 GPa |
|                                               | $Fe_{63}Cr_8Mo_2B_{17}C_5Si_1Al_4$ (DAR1) | 15.5 GPa |

15 From the hardness determined for DAR1, the yield strengths for the DNC steel can be estimated to be 725 ksi, which is significantly higher than conventional (150 ksi) or ultra high strength (220 ksi) steels. If the plasticity is fully developed, the yield strength can be estimated to be  $\frac{1}{3}$  of the hardness. This gives the DNC steel a specific strength of 20  $0.65 \times 10^6 M$  which makes this material an alternate for Al in lightweight applications. Little hardness difference was 25 found between the large and small heated powders indicating that similar microstructures were obtained independent of powder size. It is noted that the hardness tests described herein were relative to a material DAR1 ( $Fe_{63}Cr_8Mo_2B_{17}C_5Si_1Al_4$ ) which is not a preferred material of the present invention. Rather, preferred materials of the present invention would have fewer elements, and are listed as DAR2 through DAR 19 in Table 1.

30 A preferred material of the present invention (specifically DAR20) is compared with DAR1 in FIG. 11. Specifically, Vickers microhardness measurements with a 100 gram load were performed on 75 micrometer to 100 micrometer powder size fractions for as-atomized alloys, and also as a function of heat treatment temperature. The tested alloys exhibited extreme hardness from 10.1 GPa to 16.0 GPa 35 Vickers hardness. Examples of diamond pyramid indentations on a melt-spun ribbon and gas-atomized powder particle are shown in FIG. 12. While the Rockwell C is the most common hardness measurement for steels, it cannot be used in the present case due to the extreme hardness of the alloys of the present invention (which are off of the Rockwell C scale). Note that a Vickers Hardness number of 9.2 GPa corresponds to a Rockwell C of 68. Referring again to FIG. 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 865

Metallographic examinations of the coatings indicate that the percent porosity of the initial coatings was at least 3%. X-ray diffraction scans were performed both on the substrate side and free surface side of the coatings, and show that an amorphous structure was obtained through the cross-sectioning of the coatings (specifically, FIG. 14 shows an x-ray structure of a free surface side of the coating, and FIG. 15 shows an x-ray structure of the substrate side of the coating). Differential scanning calorimetry methods verified the formation of the glass structure in the coating which exhibited a high crystallization enthalpy (-110 J/g). This result is surprising due to the supreme thickness of the coating which resulted from successive build-up of continuous layers of deposited powder, and the fact that the substrate was not cooled. Thus, DNC steel coatings represent a class of materials called bulk glasses. Bulk glasses are normally very difficult to produce, but readily form in the DNC alloys by thermal processing methods.

The as-sprayed DNC metallic glass coatings can be devitrified into a nanoscale structure by heating above the crystallization temperature. However, due to the unique properties of the metallic glasses, the glass state itself may be useful as a coating. Metallic glasses are essentially super-cooled liquids, and have structures which are very homogeneous. Typically there are few defects, and there can be a complete absence of grains and phase boundaries. Hardness testing was performed on both the as-sprayed (amorphous) and heat-treated (800° C. for one hour) nanocrystalline coatings. The Vickers hardness of these coatings was found to be 10.9 GPa and 13.8 GPa for the as-sprayed and heat-treated coatings, respectively. It is noted that while the amorphous sample is not as hard as the crystalline sample, it is still harder than the hardest tool steel (about 9.3 GPa), or tungsten carbon (WC) cemented carbide cutting tool (about 10.0 GPa).

Tribology testing experiments were done on the as-sprayed and heat-treated (100° C. for one hour) plasma sprayed coatings using ASTM G99 Pin-on-Disk tests. The "pin" was a one-half inch diameter  $\text{Si}_3\text{N}_4$  ball which was rotated at a test speed of 97 RPM, with a test radius of 10.4 mm and with no lubrication. During the test, the coefficients of friction were measured (shown in FIG. 16). The coefficient of static friction for the steel substrate in both the as-sprayed and heat-treated condition was 0.22, which represents a low value. For example, the following coefficients of sliding friction were obtained for specimens sliding over a normalized steel (0.13% C, 3.42% Ni): aluminum (0.6), cartridge brass (0.5), copper (0.8), cast iron (0.4), and normalized steel (on itself 0.8). For conventional steels, the coefficients of static friction for unlubricated surfaces generally vary from 0.8 to 1.0, while lubricated steels have much lower values (typically from 0.1 to 0.25). Thus, the unlubricated DNC steels have coefficients of static friction in the range of lubricated steel surfaces. Accordingly, utilization of DNC steel coatings in place of conventional steel may allow the elimination of lubrication in some applications. Note that the coefficient of sliding friction of the steel substrate could not be measured due to  $\text{Si}_3\text{N}_4$  deposition from the pin.

The profile of the wear surface of the steel showed that the steel experienced no wear during the test (FIG. 17). Instead of the expected wear groove, a raised hill of deposited  $\text{Si}_3\text{N}_4$  was found on the steel surface. Examination of the silicon nitride ball showed that it experienced a large ball scar as a result of wear. This was surprising due to the hardness of the ball material (15.4 GPa), which is used specifically for these type of tests due to its excessive hardness and wear resis-

tance. Note that  $\text{Si}_3\text{N}_4$  is currently the hardest pin material available to perform this ASTM test.

The  $\text{Fe}_{63}\text{Cr}_8\text{Mo}_2\text{B}_{17}\text{C}_5\text{Si}_1\text{Al}_4$  steel utilized in generating the data described above is an exemplary DNC steel. However, it suffers from a disadvantage of having numerous elements included therein, which can make it difficult to produce uniform batches of the material. Accordingly, improved DNC alloys have been developed. Such improved alloys are listed in Table 1 as DAR2 through DAR19. The 10 alloys have been designed to form metallic glasses at low cooling rates, and are further designed to reduce the number of elements utilized in the alloys.

Ingots of the 19 alloys listed in Table 1 were melt-spun at 15 m/s with the following melt-spinning parameters: chamber  $\frac{1}{3}$  atmosphere helium, ejection pressure 150 Torr, ejection temperature 1,400° C., crucible up to wheel distance 6 mm, and crucible orifice diameter 0.81 mm to 0.84 mm.

All of the tested alloys were melt-spun with few problems. Interestingly, many of the preferred alloys (i.e., DAR2 20 through DAR19) formed uniform continuous ribbons up to 10 meters in length. This may be due to increased glass forming ability and increased ductility of the glass that is produced relative to the less preferred alloy DAR1. Qualitative inspections of the ribbons by bending the ribbons back 25 and forth until fracture indicated that all of the alloys DAR2 through DAR19 have higher ductility than the DAR1 alloy. In fact, some of the alloys DAR2 through DAR 19 in ribbon-form cannot be broken by bending, and had to be cut. An example of a melt-spun ribbon which exhibits high 30 ductility is shown in FIG. 18, and was formed from the material DAR18 ( $\text{Fe}_{0.8}\text{Cr}_{0.2}\text{B}_{17}\text{W}_2$ ).

Differential thermal analysis (DTA) and differential thermal calorimetry (DSC) studies were done on each melt-spun ribbon sample in ultra-high purity argon from 30° C. to 35 1,375° C. at a heating rate of 10° C./min. A typical DTA scan showing DAR14 ( $(\text{Fe}_{0.8}\text{Cr}_{0.2})_{75}\text{B}_{17}\text{Si}_4\text{Al}_4$ ) compared with DAR1 ( $\text{Fe}_{63}\text{Cr}_8\text{Mo}_2\text{B}_{17}\text{C}_5\text{Si}_1\text{Al}_4$ ) is illustrated in FIG. 19. From the DTA/DSC studies, the glass to crystalline transformation temperatures, enthalpy of transformation, transformation rate, and melting temperatures could be determined. The results of these studies are shown in FIGS. 20-23. As shown, all of the alloys but one (specifically, 40 DAR5 ( $(\text{Fe}_{0.8}\text{Mo}_{0.2})_{83}\text{B}_{17}$ )), formed a metallic glass structure when melt-spun at reduced cooling rate. Thus, the alloys are 45 expected to form metallic glass powders when atomized.

Vickers hardness testing using a 100 gram load was done on the cross-sections of the melt-spun ribbons of each alloy in the as-spun and heat-treated (700° C. for one hour and 50 800° C. for one hour) conditions. For each sample (60 samples total), 10 Vickers hardness tests on five ribbons were done in order to get a reportable average value. In general, only small variations were found to occur in hardness when the same sample was tested. Summaries of the 55 completed Vickers hardness measurements are shown in Table 4.

TABLE 4

| ALLOY                                                  | Condition | Hardness (kg/mm <sup>2</sup> ) | Hardness (GPa) |
|--------------------------------------------------------|-----------|--------------------------------|----------------|
| $(\text{Fe}_{0.85}\text{Cr}_{0.15})_{83}\text{B}_{17}$ | As-Spun   | 996                            | 9.77           |
| $(\text{Fe}_{0.85}\text{Cr}_{0.15})_{83}\text{B}_{17}$ | 700° C.   | 835                            | 8.19           |
| $(\text{Fe}_{0.85}\text{Cr}_{0.15})_{83}\text{B}_{17}$ | 800° C.   | 864                            | 8.47           |
| $(\text{Fe}_{0.8}\text{Cr}_{0.2})_{83}\text{B}_{17}$   | As-Spun   | 1048                           | 10.28          |
| $(\text{Fe}_{0.8}\text{Cr}_{0.2})_{83}\text{B}_{17}$   | 700° C.   | 935                            | 9.17           |
| $(\text{Fe}_{0.8}\text{Cr}_{0.2})_{83}\text{B}_{17}$   | 800° C.   | 870                            | 8.53           |
| $(\text{Fe}_{0.75}\text{Cr}_{0.25})_{83}\text{B}_{17}$ | As-Spun   | 1065                           | 10.45          |

TABLE 4-continued

| ALLOY                                                                                                              | Condition | Hardness (kg/mm <sup>2</sup> ) | Hardness (GPa) |
|--------------------------------------------------------------------------------------------------------------------|-----------|--------------------------------|----------------|
| (Fe <sub>0.75</sub> Cr <sub>0.25</sub> ) <sub>83</sub> B <sub>17</sub>                                             | 700° C.   | 1011                           | 9.91           |
| (Fe <sub>0.75</sub> Cr <sub>0.25</sub> ) <sub>83</sub> B <sub>17</sub>                                             | 800° C.   | 888                            | 8.71           |
| (Fe <sub>0.6</sub> Co <sub>0.2</sub> Cr <sub>0.2</sub> ) <sub>83</sub> B <sub>17</sub>                             | As-Spun   | 980                            | 9.61           |
| (Fe <sub>0.6</sub> Co <sub>0.2</sub> Cr <sub>0.2</sub> ) <sub>83</sub> B <sub>17</sub>                             | 700° C.   | 1119                           | 10.97          |
| (Fe <sub>0.6</sub> Co <sub>0.2</sub> Cr <sub>0.2</sub> ) <sub>83</sub> B <sub>17</sub>                             | 800° C.   | 984                            | 9.65           |
| (Fe <sub>0.6</sub> Cr <sub>0.15</sub> Mo <sub>0.05</sub> ) <sub>83</sub> B <sub>17</sub>                           | As-Spun   | 1062                           | 10.41          |
| (Fe <sub>0.6</sub> Cr <sub>0.15</sub> Mo <sub>0.05</sub> ) <sub>83</sub> B <sub>17</sub>                           | 700° C.   | 1573                           | 15.43          |
| (Fe <sub>0.6</sub> Cr <sub>0.15</sub> Mo <sub>0.05</sub> ) <sub>83</sub> B <sub>17</sub>                           | 800° C.   | 900                            | 8.83           |
| (Fe <sub>0.8</sub> Cr <sub>0.2</sub> ) <sub>79</sub> B <sub>1</sub> γ <sub>4</sub>                                 | As-Spun   | 1103                           | 10.82          |
| (Fe <sub>0.8</sub> Cr <sub>0.2</sub> ) <sub>79</sub> B <sub>1</sub> γ <sub>4</sub>                                 | 700° C.   | 1317                           | 12.91          |
| (Fe <sub>0.8</sub> Cr <sub>0.2</sub> ) <sub>79</sub> B <sub>1</sub> γ <sub>4</sub>                                 | 800° C.   | 1194                           | 11.71          |
| (Fe <sub>0.8</sub> Cr <sub>0.2</sub> ) <sub>79</sub> B <sub>1</sub> Si <sub>4</sub>                                | As-Spun   | 1096                           | 10.75          |
| (Fe <sub>0.8</sub> Cr <sub>0.2</sub> ) <sub>79</sub> B <sub>1</sub> Si <sub>4</sub>                                | 700° C.   | 1150                           | 11.28          |
| (Fe <sub>0.8</sub> Cr <sub>0.2</sub> ) <sub>79</sub> B <sub>1</sub> Si <sub>4</sub>                                | 800° C.   | 885                            | 8.67           |
| (Fe <sub>0.8</sub> Cr <sub>0.2</sub> ) <sub>79</sub> B <sub>1</sub> Al <sub>4</sub>                                | As-Spun   | 1053                           | 10.32          |
| (Fe <sub>0.8</sub> Cr <sub>0.2</sub> ) <sub>79</sub> B <sub>1</sub> Al <sub>4</sub>                                | 700° C.   | 1119                           | 10.97          |
| (Fe <sub>0.8</sub> Cr <sub>0.2</sub> ) <sub>79</sub> B <sub>1</sub> Al <sub>4</sub>                                | 800° C.   | 946                            | 9.28           |
| (Fe <sub>0.8</sub> Cr <sub>0.2</sub> ) <sub>75</sub> B <sub>1</sub> Al <sub>4</sub> C <sub>4</sub>                 | As-Spun   | 1098                           | 10.76          |
| (Fe <sub>0.8</sub> Cr <sub>0.2</sub> ) <sub>75</sub> B <sub>1</sub> Al <sub>4</sub> C <sub>4</sub>                 | 700° C.   | 1380                           | 13.53          |
| (Fe <sub>0.8</sub> Cr <sub>0.2</sub> ) <sub>75</sub> B <sub>1</sub> Al <sub>4</sub> C <sub>4</sub>                 | 800° C.   | 1159                           | 11.37          |
| (Fe <sub>0.8</sub> Cr <sub>0.2</sub> ) <sub>75</sub> B <sub>1</sub> Al <sub>4</sub> C <sub>4</sub>                 | As-Spun   | 1184                           | 11.61          |
| (Fe <sub>0.8</sub> Cr <sub>0.2</sub> ) <sub>75</sub> B <sub>1</sub> Al <sub>4</sub> C <sub>4</sub>                 | 700° C.   | 1509                           | 14.80          |
| (Fe <sub>0.8</sub> Cr <sub>0.2</sub> ) <sub>75</sub> B <sub>1</sub> Al <sub>4</sub> C <sub>4</sub>                 | 800° C.   | 1245                           | 12.21          |
| (Fe <sub>0.8</sub> Cr <sub>0.2</sub> ) <sub>75</sub> B <sub>1</sub> Al <sub>4</sub> C <sub>4</sub>                 | As-Spun   | 1063                           | 10.42          |
| (Fe <sub>0.8</sub> Cr <sub>0.2</sub> ) <sub>75</sub> B <sub>1</sub> Al <sub>4</sub> C <sub>4</sub>                 | 700° C.   | 1266                           | 12.42          |
| (Fe <sub>0.8</sub> Cr <sub>0.2</sub> ) <sub>75</sub> B <sub>1</sub> Al <sub>4</sub> C <sub>4</sub>                 | 800° C.   | 1055                           | 10.34          |
| (Fe <sub>0.8</sub> Cr <sub>0.2</sub> ) <sub>71</sub> B <sub>1</sub> Si <sub>4</sub> C <sub>4</sub> Al <sub>4</sub> | As-Spun   | 1093                           | 10.72          |
| (Fe <sub>0.8</sub> Cr <sub>0.2</sub> ) <sub>71</sub> B <sub>1</sub> Si <sub>4</sub> C <sub>4</sub> Al <sub>4</sub> | 700° C.   | 1376                           | 13.49          |
| (Fe <sub>0.8</sub> Cr <sub>0.2</sub> ) <sub>71</sub> B <sub>1</sub> Si <sub>4</sub> C <sub>4</sub> Al <sub>4</sub> | 800° C.   | 1134                           | 11.12          |
| (Fe <sub>0.7</sub> Co <sub>0.1</sub> Cr <sub>0.2</sub> ) <sub>83</sub> B <sub>17</sub>                             | As-Spun   | 1042                           | 10.22          |
| (Fe <sub>0.7</sub> Co <sub>0.1</sub> Cr <sub>0.2</sub> ) <sub>83</sub> B <sub>17</sub>                             | 700° C.   | 1135                           | 11.13          |
| (Fe <sub>0.7</sub> Co <sub>0.1</sub> Cr <sub>0.2</sub> ) <sub>83</sub> B <sub>17</sub>                             | 800° C.   | 885                            | 8.68           |
| (Fe <sub>0.8</sub> Cr <sub>0.2</sub> ) <sub>80</sub> B <sub>20</sub>                                               | As-Spun   | 1093                           | 10.72          |
| (Fe <sub>0.8</sub> Cr <sub>0.2</sub> ) <sub>80</sub> B <sub>20</sub>                                               | 700° C.   | 1045                           | 10.24          |
| (Fe <sub>0.8</sub> Cr <sub>0.2</sub> ) <sub>80</sub> B <sub>20</sub>                                               | 800° C.   | 965                            | 9.47           |
| (Fe <sub>0.8</sub> Cr <sub>0.2</sub> ) <sub>76</sub> B <sub>1</sub> Al <sub>7</sub>                                | As-Spun   | 1028                           | 10.08          |
| (Fe <sub>0.8</sub> Cr <sub>0.2</sub> ) <sub>76</sub> B <sub>1</sub> Al <sub>7</sub>                                | 700° C.   | 1441                           | 14.13          |
| (Fe <sub>0.8</sub> Cr <sub>0.2</sub> ) <sub>76</sub> B <sub>1</sub> Al <sub>7</sub>                                | 800° C.   | 868                            | 8.51           |
| (Fe <sub>0.8</sub> Cr <sub>0.2</sub> ) <sub>79</sub> B <sub>1</sub> W <sub>2</sub> C <sub>2</sub>                  | As-Spun   | 1124                           | 11.02          |
| (Fe <sub>0.8</sub> Cr <sub>0.2</sub> ) <sub>79</sub> B <sub>1</sub> W <sub>2</sub> C <sub>2</sub>                  | 700° C.   | 1653                           | 16.21          |
| (Fe <sub>0.8</sub> Cr <sub>0.2</sub> ) <sub>79</sub> B <sub>1</sub> W <sub>2</sub> C <sub>2</sub>                  | 800° C.   | 1223                           | 11.99          |
| (Fe <sub>0.8</sub> Cr <sub>0.2</sub> ) <sub>81</sub> B <sub>1</sub> W <sub>2</sub>                                 | As-Spun   | 1052                           | 10.31          |
| (Fe <sub>0.8</sub> Cr <sub>0.2</sub> ) <sub>81</sub> B <sub>1</sub> W <sub>2</sub>                                 | 700° C.   | 1565                           | 15.34          |
| (Fe <sub>0.8</sub> Cr <sub>0.2</sub> ) <sub>81</sub> B <sub>1</sub> W <sub>2</sub>                                 | 800° C.   | 1100                           | 10.79          |

As indicated by the tables and Figures provided herein, materials of the present invention having less than 11 elements, and more preferably less than seven elements, can form glass compositions. It is not a trivial task to form materials having such limited number of elements, which are also capable of forming metallic glasses. However, such has been accomplished in the present invention. The present invention also has developed improved ductility and toughness of DNC steel alloys, while maintaining or possibly even improving hardness. The DNC alloys are believed to be useful for numerous services, including military applications, due to their strength and wear resistance. The alloys can also be resistant to electrochemical attack (i.e., corrosion). In general, as the scale of a microstructure decreases, the electrochemical resistance of a particular material is expected to increase. Thus, nanocrystalline scale DNC microstructures are expected to have good corrosion resistance. Further, metallic glass DNC structures can have improved corrosion resistance due to high homogeneity (short range order on a 2 nanometer length scale) and the absence of two-dimensional defects (such as grain or phase boundaries). Specifically, a uniform single-phase structure can make it difficult for sites to initiate for anodic attack and electron transfer since there will not be distinct anodic and cathodic sites. While the metallic glass or nanostructure of

a certain composition can have a higher relative resistance to electrochemical attack than the same material in bulk form, the material's nobility will be dependent on both the structure and the composition. For instance, a high level of chromium can improve resistance to electrochemical attack.

Among the advantages of the alloys described herein is that such alloys can have a relatively simple composition (i.e., from four to six elements in the composition). Also, the alloys can contain a relatively high percentage of transition metals (from 90% to 97%) which can lead to improved industrial properties of the materials.

A distinction of the materials of the present invention relative to conventional hard materials is that the materials of the present invention can comprise no carbon. In conventional steels, hardness is typically tied directly to carbon content in a martensite. In contrast, the extreme hardness of DNC steels arises from development of nanoscale nanocomposite microstructures, rather than from martensitic transformations. An advantage of carbon-free compositions is that the extremely hard alloys can be developed to still be reasonably ductile, which is typically not possible in conventional steel alloys (i.e., untempered martensite and transition metal carbides are typically hard, and also brittle).

Group VI transition metals (Cr, Mo, and W) can be particularly potent additions to DNC steels. Chromium, consistent with data on conventional steel alloys, is expected to also provide excellent corrosion resistance. Molybdenum and tungsten can be exceptionally potent additions to promote hardness in DNC steels. Tungsten can also be potent at increasing hardness while retaining or increasing ductility.

Because of its hardness and high strength (greater than 725 ksi), DNC steel can be difficult to process into bulk parts starting from powder and using conventional powder metallurgical consolidation processes. However, DNC steel can be easy to process from the liquid state. Alternatively, powder of DNC steel can be fed through a conventional plasma gun and sprayed as a coating onto metal substrates with good adhesion and with absence of cracking. Other methods for forming a coating of DNC steel include axial feed plasma spray, conventional plasma spray, high velocity oxy-fuel spray, and a detonation gun.

When DNC steel is sprayed onto metallic substrates it can readily form a metallic glass structure. If consecutive layers are continuously sprayed onto a bulk substrate (thickness greater than 0.1 inches) metallic glasses can be formed. This may be the most inexpensive and easiest way to form bulk metallic glass coatings or even bulk glass monolithic parts.

DNC steels can be rapidly solidified into an amorphous glass precursor and then the rapidly solidified powders can be consolidated into a useful form. Accordingly, the cost of technology of the present invention can involve three items: the alloy cost, the powder production cost, and the consolidation cost. All three items can be estimated. To produce rapidly solidified powder, centrifugal atomization may be the best method, and even at relatively low production rates. If it is feasible to produce DNC steel powder by water atomization, processing cost to produce the powder could drop to a few pennies per pound. The powder consolidation costs will vary depending on the specific application and the thickness of the coating. Coatings from 5 micrometers to 2,500 micrometers in thickness can be readily deposited using conventional commercially available thermal deposition methods, such as plasma spraying or high velocity oxy-fuel spraying. The DNC steel's cost can compare favorably to other hard materials such as, for example, diamond and cubic BN. DNC steel coating may also be a direct competing technology to replace tungsten carbide cemented

**15**

carbide coatings, since the DNC steel exhibits higher hardness and greater tensile ductility.

Although the invention is described herein for coating steel alloy compositions of the present invention on metallic substrates, it is to be understood that the alloys of the present invention can also be coated on non-metallic substrates, such as, for example, ceramics, to provide a hard and/or lubricating surface over the non-metallic substrates.

In compliance with the statute, the invention has been described in language more or less specific as to structural and methodical features. It is to be understood, however, that the invention is not limited to the specific features shown and described, since the means herein disclosed comprise preferred forms of putting the invention into effect. The invention is, therefore, claimed in any of its forms or modifications within the proper scope of the appended claims appropriately interpreted in accordance with the doctrine of equivalents.

The invention claimed is:

1. A method of forming a hardened surface on a substrate, comprising:
  - 10 providing a substrate; and
  - 15 forming a molten alloy and cooling said alloy to form a metallic glass coating on the substrate, the forming comprising forming a successive buildup of metallic glass layers, the metallic glass coating having a hardness of at least about 9.2 GPa, and comprising an alloy consisting of at least 50% iron, optionally chromium, one or more elements selected from the group consisting of boron and phosphorous, one or both of molybdenum and tungsten; and at least one member of the group consisting of Ga, Ge, Au, Zr, Hf, Nb, Ta, La, Ce, Pr, Nd, Sm, Eu, Gd, Tb, Dy, Ho, Er, Tm, Yb, Lu, N, S, and O.
  - 20 2. The method of claim 1 wherein the substrate is a metallic material.
  - 25 3. The method of claim 1 wherein the substrate is a ceramic material.

**16**

4. The method of claim 1 wherein the metallic glass coating is applied to the substrate as a plasma spray.

5. The method of claim 1 wherein the forming the metallic glass coating comprises an application of an atomized powder of a metallic glass material over the substrate.

6. A method of forming a hardened surface on a substrate, comprising:

providing a substrate; and  
 forming a molten alloy and cooling said alloy to form a metallic glass coating on the substrate and having a first hardness of at least about 9.2 GPa, the metallic glass consisting of at least 50% iron, optionally chromium, one or more elements selected from the group consisting of boron and phosphorous, and at least one member of the group consisting of Ga, Ge, Au, Zr, Hf, Nb, Al, La, Ce, Pr, Nd, Sm, Eu, Gd, Tb, Dy, Ho, Er, Tm, Yb, Lu, N, S, and O; and converting at least a portion of the metallic glass coating to a crystalline material having a nanocrystalline grain size and a second hardness of at least about 9.2 GPa.

7. The method of claim 6 wherein the first hardness is at least about 10.0 GPa.

8. The method of claim 6 wherein the forming a metallic glass coating comprises forming a successive buildup of continuous layers.

9. The method of claim 6 wherein the converting comprises heating the metallic glass to above a crystallization temperature of the metallic glass.

10. The method of claim 9 wherein the heating comprises heating to a temperature of at least about 600° C. and below a melting temperature of the metallic glass.

11. The method of claim 6 wherein the second hardness is at least about 10.0 GPa.

12. The method of claim 6 wherein the forming the hardened surface comprises an application of an atomized powder of a metallic glass material over the substrate.

\* \* \* \* \*